

# United States Patent Office

3,736,098  
Patented May 29, 1973

1

3,736,098  
METHOD OF INHIBITING THE ACID  
CORROSION OF METALS

Toshiya Kataoka, Chigasaki-shi, and Atunobu Takada,  
Tokyo, Japan, assignors to Nissin Oil Mills, Ltd.,  
Tokyo, Japan  
No Drawing. Filed Jan. 18, 1972, Ser. No. 218,825  
Int. Cl. C23f 11/14

U.S. Cl. 21—2.7 R

9 Claims

### ABSTRACT OF THE DISCLOSURE

A method of preventing the acid corrosion of metals which consists in inhibiting acid solutions from corroding metals by mixing with said acid solutions an anticorrosive composition prepared by the reaction of benzyl halides and materials mainly consisting of imidazoline derivatives having the following structural formula:



where:

R=an alkyl, alkenyl or hydroxyalkenyl radical having 5 to 21 carbon atoms  
m=0 or integer of 1 to 3

### BACKGROUND OF THE INVENTION

This invention relates to a method of inhibiting metals from being corroded by acids and anticorrosive agents for metals.

It is generally known that compounds of the imidazoline series are effective to inhibit metals from being corroded by acids. Said effect primarily consists in inhibiting the surface of metals from being tarnished brown when they are in contact with, for example, a solution of hydrochloric acid.

Where 1-(2'-aminoethyl)-2-alkyl (or alkenyl) imidazoline is used as an anticorrosive agent in subjecting metals to acid washing, said agent displays an effect of considerably preventing metals from being tarnished brown, in case the washing acid consists of hydrochloric acid. However, said anticorrosive agent is still deemed unsatisfactory to inhibit the corrosion weight loss of metals. Further, where there is used a hot washing acid solution over a long period, the anticorrosive agent contained therein presents a reduced effect due to its own hydrolysis, failing to be applied at all depending on the object of acid washing.

### SUMMARY OF THE INVENTION

The present inventors have discovered that where 1-(2'-aminoethyl)-2-alkyl (or alkenyl) imidazoline is reacted with benzyl halides to convert the valency of the nitrogen constituting an imidazoline ring to a tetravalent form, thereby obtaining imidazolinium salts, and the benzyl group is also introduced into the aminoethyl group, then the resultant composition has a far more excellent property of inhibiting metals from being corroded by an acid solution than the original 1-(2'-aminoethyl)-2-alkyl (or alkenyl) imidazoline alone.

This invention has been accomplished from the above-mentioned discovery. According to one aspect of the invention, there is provided a method of inhibiting acid solutions from corroding metals by mixing said acid solu-

2

tions with an anticorrosive composition prepared by the reaction of benzyl halides and materials mainly consisting of imidazoline derivatives having the following structural formula:



10 where:

R=group of alkyl, alkenyl or hydroxyalkenyl having 5 to 21 carbon atoms  
m=0 or integer of 1 to 3

15 According to another aspect of the invention, there is provided a method of inhibiting acid solutions from corroding metals by adding to said solutions not only an anticorrosive composition prepared by the reaction of benzyl halides and materials mainly consisting of imidazoline derivatives having the above-mentioned structural formula but also an additive capable of prominently promoting the solubility of said anticorrosive agent in acid solutions.

20 This invention far more reduces the weight loss of metals caused by acid corrosion than has been possible with the prior art, thereby fully protecting the metals from corrosion by hot acid solutions even when the metals are exposed thereto for long hours.

### DETAILED DESCRIPTION OF THE INVENTION

25 Imidazoline derivatives used as the raw material of the subject anticorrosive composition can be prepared by reacting fatty acids with polyethylene polyamines such as diethylene triamine (DETA), triethylene tetramine (TETA), tetraethylene pentamine (TEPA) and pentaethylene hexamine (PEHA) by the ordinary process according to the following Equation 1:



where:

45 R=group of alkyl, alkenyl or hydroxyalkenyl  
x=integer of 1 to 4  
m=0 or integer of 1 to 3.

50 The above remark applies hereinafter. However, according as x of the general formula of polyethylene polyamines indicated in the Equation 1 above has an increasing value, there unavoidably occur as byproduct small amounts of imidazoline derivatives expressed by the following structural Formulas A and B:



55 where: p=0 or integer of 1 or 2.

3

Since, however, the main component of said anticorrosive composition is substantially formed of a type represented by the structural formula shown in the reaction Formula 1, it is preferred for economic reason to use said composition in a state mixed with such byproducts expressed by the structural Formulas A and B instead of particularly separating them.

The anticorrosive composition of the Equation 1 may also be prepared by any desired process according to either of the following Equation 2 or 3.



Reaction of imidazoline derivatives with, for example, benzyl chloride included in the aforesaid benzyl halides easily proceeds by applying heat at a temperature of 60 to 150° C., or preferably 80 to 120° C.

The proportion of the benzyl halide which is to be reacted with the imidazoline derivatives should preferably be limited to such extent that the amount of said benzyl halide does not exceed an equivalent to the number of reactive imidazoline rings and amino groups contained in the molecule of the imidazoline derivatives, namely, that there do not remain large amounts of unreacted benzyl halide after completion of reaction.

Reaction of the imidazoline derivatives with the benzyl halide may be expressed by combinations of the following Equations 4 to 8, the resultant composition being formed of various mixtures of the reaction products.



fore reacted with benzyl halides are easily subject to hydrolysis by a hot acid solution, the main component of the present anticorrosive composition consists of imidazolinium salts converted to a tetravalent form by being reacted with benzyl halides and consequently is little hydrolyzed even when mixed with a hot acid solution, retaining an anticorrosive effect over a long period.

Referring to the alkyl or alkenyl group contained in the anticorrosive composition of this invention, the type having 5 to 21 carbon atoms is effective. Also effective is the alkenyl group containing a hydroxyl group derived from ricinoleic acid. This type of alkenyl group has a hydrophilic hydroxyl group positioned at the intermediate part of a carbon chain and consequently is characterized by rendering the anticorrosive composition less frothy.

When added to an acid solution, the anticorrosive composition of this invention which originally has low solubility therein naturally makes the solution turbid. Since, however, the composition is well dispersed, said turbidity itself does not normally exert a harmful effect on the anticorrosive effect of said composition, but enables it fully to protect metals from acid corrosion.

There are occasions, however, where an acid solution is not desired to be cloudy. In such case, the anticorrosive composition should be made sufficiently soluble in said acid solution to maintain its transparency when mixed therewith. A solubilizer added to this end is required to be stable to an acid solution and free from a harmful effect on the protection of metals from acid corrosion. Economically favorable are such solubilizers as ethylene oxide addition product of higher alcohols, alkyl phenols and alkyl amines. Where, therefore, the anticorrosive composition is used with a hot acid solution it is preferred that said composition be mixed with solubilizer for example, ethylene oxide addition product of alkyl amines which does not cause the acid solution to present a cloud point.

The present invention will be more fully understood by reference to the examples which follow.

#### EXAMPLE 1

There were used the following types of anticorrosive composition.

- (I) 1-(2'-aminoethyl)-2-cocoimidazoline
- (I-A) A composition prepared by the reaction with 0.5 mol of benzyl chloride added based on 1.0 mol of the Type I
- (I-B) A composition prepared by the reaction with 1.0 mol of benzyl chloride added based on 1.0 mol of the Type I
- (I-C) A composition prepared by the reaction with 1.5 mol of benzyl chloride added based on 1.0 mol of the Type I
- (I-D) A composition prepared by the reaction with 2.0 mol of benzyl chloride added based on 1.0 mol of the Type I
- (I-E) A composition prepared by the reaction with 2.0 mol of benzyl iodide added based on 1.0 mol of the Type I
- (II) 1-(2'-aminoethyl)-2-rapeimidazoline
- (II-A) A composition prepared by the reaction with 2.0 mol of benzyl chloride added based on 1.0 mol of the Type II
- (III) 1-(2'-aminoethyl)-2-castorimidazoline
- (III-A) A composition prepared by the reaction with 2.0 mol of benzyl chloride added based on 1.0 mol of the Type III
- (IV) 1-2-(2'-aminoethyl)aminoethyl-2-undecyl imidazoline
- (IV-A) A composition prepared by the reaction with 2.0 mol of benzyl chloride added based on 1.0 mol of the Type IV
- (V) An imidazoline derivative prepared from lauric acid and TEPA
- (V-A) A composition prepared by the reaction with

- 2.0 mol of benzyl chloride added based on 1.0 mol of the Type V
- (V-B) A composition prepared by the reaction with 3.0 mol of benzyl chloride added based on 1.0 mol of the Type V
- (VI) An imidazoline derivative prepared from lauric acid and PEHA
- (VI-A) A composition prepared by the reaction with 3.0 mol of benzyl chloride added based on 1.0 mol of the Type VI
- (VI-B) A composition prepared by the reaction with 4.0 mol of benzyl chloride added based on 1.0 mol of the Type VI

15 Among the above-listed corrosive compositions, those of the Types I, II, III, IV, V and VI only consist of imidazoline derivatives which were not reacted with benzyl halides. They were used simply as controls or reference samples in the tests of determining the capacity to prevent acid corrosion in order to distinguish more clearly the effect of anticorrosive compositions of this invention.

20 Cold pressed milled steel coupons (50 mm. x 20 mm. x 2 mm.) were submerged in 150 ml. of 7% hydrochloric acid solutions to which there were added prescribed amount of anticorrosive composition. The coupons were allowed to stand in said acid solutions for 5 hours at a 25 temperature of 70° C. to measure their corrosion rates (mg./cm.<sup>2</sup>/hr.). At the same time there were conducted blank tests with 7% pure hydrochloric acid solution. The 30 percentage inhibition efficiency acid corrosion was determined by the following equation.

$$35 \text{ Percent inhibition efficiency} = \frac{B-A}{B} \times 100$$

40 where:

A=corrosion rate with addition of an anticorrosive composition

B=corrosion rate in a blank test

45 The results of the corrosion inhibition tests are presented in Tables 1, 2 and 3 below.

50 TABLE 1.—CORROSION INHIBITING EFFECT  
[7% HCl, 70° C., 5 hr.]

| Anticorrosive composition |       | Type   | Amount added, percent | Corrosion rate, mg./cm. <sup>2</sup> /hr.               | Inhibition efficiency, percent | Surface of processed steel coupon |
|---------------------------|-------|--------|-----------------------|---------------------------------------------------------|--------------------------------|-----------------------------------|
|                           |       |        |                       |                                                         |                                |                                   |
| I-----                    | 0.010 | 0.484  | 97.7                  | Maintains the original metal luster.                    |                                |                                   |
| I-----                    | 0.025 | 0.209  | 99.0                  | Do.                                                     |                                |                                   |
| I-----                    | 0.050 | 0.185  | 99.1                  | Do.                                                     |                                |                                   |
| I-A-----                  | 0.050 | 0.170  | 99.2                  | Do.                                                     |                                |                                   |
| I-B-----                  | 0.010 | 0.205  | 99.0                  | Do.                                                     |                                |                                   |
| I-B-----                  | 0.025 | 0.118  | 99.4                  | Do.                                                     |                                |                                   |
| I-B-----                  | 0.050 | 0.100  | 99.5                  | Do.                                                     |                                |                                   |
| I-C-----                  | 0.010 | 0.172  | 99.2                  | Do.                                                     |                                |                                   |
| I-C-----                  | 0.025 | 0.105  | 99.5                  | Do.                                                     |                                |                                   |
| I-C-----                  | 0.050 | 0.092  | 99.6                  | Do.                                                     |                                |                                   |
| I-D-----                  | 0.010 | 0.186  | 99.1                  | Do.                                                     |                                |                                   |
| I-D-----                  | 0.025 | 0.109  | 99.5                  | Do.                                                     |                                |                                   |
| I-D-----                  | 0.050 | 0.092  | 99.6                  | Do.                                                     |                                |                                   |
| I-E-----                  | 0.010 | 0.190  | 99.1                  | Do.                                                     |                                |                                   |
| I-E-----                  | 0.025 | 0.110  | 99.5                  | Do.                                                     |                                |                                   |
| I-E-----                  | 0.050 | 0.095  | 99.6                  | Do.                                                     |                                |                                   |
| I-E-----                  | 0     | 20.936 | 0                     | Presents a dark brown color due to occurrence of smuts. |                                |                                   |

TABLE 2.—CORROSION INHIBITING EFFECT  
[7% HCl, 70° C., 5 hr.]

| Anticorrosive composition |                       | Corrosion rate, mg./cm. <sup>2</sup> /hr. | Inhibition efficiency, percent | Surface of processed steel coupon                       |
|---------------------------|-----------------------|-------------------------------------------|--------------------------------|---------------------------------------------------------|
| Type                      | Amount added, percent |                                           |                                |                                                         |
| II                        | 0.010                 | 0.358                                     | 98.3                           | Maintains the original metal luster.                    |
| II                        | 0.025                 | 0.259                                     | 98.8                           | Do.                                                     |
| II                        | 0.050                 | 0.269                                     | 98.7                           | Do.                                                     |
| II-A                      | 0.025                 | 0.144                                     | 99.3                           | Do.                                                     |
| II-A                      | 0.050                 | 0.114                                     | 99.5                           | Do.                                                     |
| III                       | 0.010                 | 0.514                                     | 97.5                           | Do.                                                     |
| III                       | 0.025                 | 0.365                                     | 98.3                           | Do.                                                     |
| III                       | 0.050                 | 0.317                                     | 98.5                           | Do.                                                     |
| III-A                     | 0.010                 | 0.135                                     | 99.4                           | Do.                                                     |
| III-A                     | 0.025                 | 0.096                                     | 99.5                           | Do.                                                     |
| III-A                     | 0.050                 | 0.114                                     | 99.5                           | Do.                                                     |
| IV                        | 0.010                 | 0.422                                     | 98.0                           | Do.                                                     |
| IV                        | 0.025                 | 0.346                                     | 98.4                           | Do.                                                     |
| IV                        | 0.050                 | 0.313                                     | 98.5                           | Do.                                                     |
| IV-A                      | 0.010                 | 0.155                                     | 99.3                           | Do.                                                     |
| IV-A                      | 0.025                 | 0.120                                     | 99.4                           | Do.                                                     |
| IV-A                      | 0.050                 | 0.110                                     | 99.5                           | Do.                                                     |
| 0                         |                       | 20.936                                    | 0                              | Presents a dark brown color due to occurrence of smuts. |

## EXAMPLE 2

5 There were heated to 80° C. the 10% hydrochloric acid solutions to which there were added a prescribed amount of the anticorrosive compositions of the Types I and 10 I-D used in Example 1. Said hydrochloric acid solutions were preserved at said temperature for 5, 10 and 30 days respectively. Thereafter, there were submersed, as in Example 1, mild steel coupons for 5 hours in said 10% hydrochloric acid solutions. There were conducted corrosion inhibition tests with said acid solutions kept at 70° C. to determine the corrosion rate and inhibition efficiency and compare the high temperature stability of the respective samples, the results being presented in Table 15 20 4 below.

25

TABLE 4.—CORROSION INHIBITING EFFECT

[10% HCl, 70° C., 5 hr.]

| Anticorrosive composition |                       | Number of days during which HCl remained mixed with anticorrosive compositions (80° C.) |                                |                                           |                                |                                           |                                |                                           |                                |
|---------------------------|-----------------------|-----------------------------------------------------------------------------------------|--------------------------------|-------------------------------------------|--------------------------------|-------------------------------------------|--------------------------------|-------------------------------------------|--------------------------------|
| Type                      | Amount added, percent | 0 days                                                                                  |                                | 5 days                                    |                                | 10 days                                   |                                | 30 days                                   |                                |
|                           |                       | Corrosion rate, mg./cm. <sup>2</sup> /hr.                                               | Inhibition efficiency, percent | Corrosion rate, mg./cm. <sup>2</sup> /hr. | Inhibition efficiency, percent | Corrosion rate, mg./cm. <sup>2</sup> /hr. | Inhibition efficiency, percent | Corrosion rate, mg./cm. <sup>2</sup> /hr. | Inhibition efficiency, percent |
| I                         | 0.010                 | 0.690                                                                                   | 97.3                           | 1.387                                     | 94.6                           | 2.020                                     | 92.2                           | -----                                     | -----                          |
| I                         | 0.025                 | 0.749                                                                                   | 97.1                           | 1.189                                     | 95.3                           | 1.371                                     | 94.7                           | -----                                     | -----                          |
| I                         | 0.050                 | 0.752                                                                                   | 97.1                           | 1.245                                     | 95.1                           | 1.438                                     | 94.4                           | -----                                     | -----                          |
| I-D                       | 0.010                 | 0.119                                                                                   | 99.5                           | 0.117                                     | 99.5                           | 0.111                                     | 99.6                           | 0.367                                     | 98.6                           |
| I-D                       | 0.025                 | 0.106                                                                                   | 99.6                           | 0.112                                     | 99.6                           | 0.153                                     | 99.4                           | 0.215                                     | 99.2                           |
| I-D                       | 0.050                 | 0.109                                                                                   | 99.6                           | 0.138                                     | 99.5                           | 0.113                                     | 99.6                           | 0.159                                     | 99.4                           |
| 0                         |                       | 25.932                                                                                  | 0                              | 25.514                                    | 0                              | 25.766                                    | 0                              | 26.576                                    | 0                              |

## EXAMPLE 3

TABLE 3.—CORROSION INHIBITING EFFECT  
[7% HCl, 70° C., 5 hr.]

| Anticorrosive composition |                       | Corrosion rate, mg./cm. <sup>2</sup> /hr. | Inhibition efficiency, percent | Surface of processed steel coupon                       |
|---------------------------|-----------------------|-------------------------------------------|--------------------------------|---------------------------------------------------------|
| Type                      | Amount added, percent |                                           |                                |                                                         |
| V                         | 0.010                 | 0.362                                     | 98.3                           | Maintains the original metal luster.                    |
| V                         | 0.025                 | 0.277                                     | 98.7                           | Do.                                                     |
| V                         | 0.050                 | 0.260                                     | 98.8                           | Do.                                                     |
| V-A                       | 0.010                 | 0.230                                     | 98.9                           | Do.                                                     |
| V-A                       | 0.025                 | 0.170                                     | 99.2                           | Do.                                                     |
| V-A                       | 0.050                 | 0.168                                     | 99.2                           | Do.                                                     |
| V-B                       | 0.010                 | 0.237                                     | 98.9                           | Do.                                                     |
| V-B                       | 0.025                 | 0.183                                     | 99.1                           | Do.                                                     |
| V-B                       | 0.050                 | 0.172                                     | 99.2                           | Do.                                                     |
| VI                        | 0.010                 | 0.490                                     | 97.7                           | Do.                                                     |
| VI                        | 0.025                 | 0.405                                     | 98.1                           | Do.                                                     |
| VI                        | 0.050                 | 0.402                                     | 98.1                           | Do.                                                     |
| VI-A                      | 0.010                 | 0.356                                     | 98.3                           | Do.                                                     |
| VI-A                      | 0.025                 | 0.266                                     | 98.7                           | Do.                                                     |
| VI-A                      | 0.050                 | 0.128                                     | 99.4                           | Do.                                                     |
| VI-B                      | 0.010                 | 0.350                                     | 98.3                           | Do.                                                     |
| VI-B                      | 0.025                 | 0.232                                     | 98.9                           | Do.                                                     |
| VI-B                      | 0.050                 | 0.245                                     | 98.8                           | Do.                                                     |
| 0                         |                       | 20.936                                    | 0                              | Presents a dark brown color due to occurrence of smuts. |

50 There were submerged mild steel coupons in 150 mol of the 10% sulfuric acid solutions to which there were added a prescribed amount of the anticorrosive compositions of the Types I and I-E used in Example 1. The steel plate was allowed to stand 2 hours in said sulfuric acid solution kept at a temperature of 60° C. Determination was made of the corrosion rate and inhibition efficiency, the results being presented in Table 5 below.

TABLE 5.—CORROSION PREVENTION EFFECT  
[10% H<sub>2</sub>SO<sub>4</sub>, 60° C., 2 hr.]

| Anticorrosive composition |                       | Corrosion rate, mg./cm. <sup>2</sup> /hr. | Inhibition efficiency, percent | Surface of processed steel coupon                        |
|---------------------------|-----------------------|-------------------------------------------|--------------------------------|----------------------------------------------------------|
| Type                      | Amount added, percent |                                           |                                |                                                          |
| I                         | 0.010                 | 3.45                                      | 75.0                           | Presented a dark brown color due to occurrence of smuts. |
| I                         | 0.025                 | 2.71                                      | 80.3                           | Do.                                                      |
| I                         | 0.050                 | 1.91                                      | 86.1                           | Do.                                                      |
| I-E                       | 0.010                 | 0.27                                      | 98.0                           | Maintains the original metal luster.                     |
| I-E                       | 0.025                 | 0.14                                      | 99.0                           | Do.                                                      |
| I-E                       | 0.050                 | 0.07                                      | 99.5                           | Do.                                                      |
| 0                         |                       | 13.77                                     | 0                              | Presents a dark brown color due to occurrence of smuts.  |

75

9  
EXAMPLE 4

There were performed corrosion inhibition tests with the anticorrosive compositions of the Types I, I-A, I-B, I-C, I-D, II, II-A, III, III-A, IV, IV-A, V, V-A, V-B, VI, VI-A and VI-B with the following types of solubilizer added:

(A) Ethylene oxide addition product of lauryl alcohol having 25 mol of ethylene oxide per 1.0 mol of lauryl alcohol.

(B<sub>1</sub>) Ethylene oxide addition product of nonyl phenol having 15 mol of ethylene oxide per 1.0 mol of nonyl phenol.

(B<sub>2</sub>) Ethylene oxide addition product of nonyl phenol having 20 mol of ethylene oxide per 1.0 mol of nonyl phenol.

(C<sub>1</sub>) Ethylene oxide addition product of stearylamine having 15 mol of ethylene oxide per 1.0 mol of stearylamine.

(C<sub>2</sub>) Ethylene oxide addition product of stearylamine having 20 mol of ethylene oxide per 1.0 mol of stearylamine.

The results are presented in Tables 6, 7 and 8 below. Through the tests there was used a transparent hydrochloric acid solution free from turbidity.

## 10

TABLE 7.—CORROSION INHIBITING EFFECT  
[7% HCl, 70° C., 5 hr.]

| Type  | Anticorrosive composition |                       | Solubilizer/amount added, percent | Corrosion rate, mg./cm. <sup>2</sup> /hr. | Inhibition efficiency, percent | Inhibition efficiency, percent       | Surface of processed steel coupon                       |
|-------|---------------------------|-----------------------|-----------------------------------|-------------------------------------------|--------------------------------|--------------------------------------|---------------------------------------------------------|
|       | Amount added, percent     | Percent               |                                   |                                           |                                |                                      |                                                         |
| II    | 0.010                     | 0                     | 0                                 | 0.358                                     | 98.3                           | Maintains the original metal luster. |                                                         |
| II    | 0.025                     | 0                     | 0                                 | 0.259                                     | 98.8                           | Do.                                  |                                                         |
| II    | 0.050                     | 0                     | 0                                 | 0.269                                     | 98.7                           | Do.                                  |                                                         |
| II-A  | 0.010                     | C <sub>1</sub> /0.002 | 0                                 | 0.087                                     | 99.6                           | Do.                                  |                                                         |
| II-A  | 0.025                     | C <sub>1</sub> /0.025 | 0                                 | 0.089                                     | 99.6                           | Do.                                  |                                                         |
| II-A  | 0.050                     | C <sub>1</sub> /0.010 | 0                                 | 0.086                                     | 99.6                           | Do.                                  |                                                         |
| III   | 0.010                     | 0                     | 0                                 | 0.514                                     | 97.5                           | Do.                                  |                                                         |
| III   | 0.025                     | 0                     | 0                                 | 0.365                                     | 98.3                           | Do.                                  |                                                         |
| III   | 0.050                     | 0                     | 0                                 | 0.317                                     | 98.5                           | Do.                                  |                                                         |
| III-A | 0.010                     | C <sub>1</sub> /0.002 | 0                                 | 0.106                                     | 99.5                           | Do.                                  |                                                         |
| III-A | 0.025                     | C <sub>1</sub> /0.005 | 0                                 | 0.111                                     | 99.5                           | Do.                                  |                                                         |
| III-A | 0.050                     | C <sub>1</sub> /0.010 | 0                                 | 0.116                                     | 99.5                           | Do.                                  |                                                         |
| IV-A  | 0.010                     | 0                     | 0                                 | 0.422                                     | 98.0                           | Do.                                  |                                                         |
| IV-A  | 0.025                     | 0                     | 0                                 | 0.346                                     | 98.4                           | Do.                                  |                                                         |
| IV-A  | 0.050                     | 0                     | 0                                 | 0.313                                     | 99.3                           | Do.                                  |                                                         |
| IV-A  | 0.010                     | C <sub>1</sub> /0.002 | 0                                 | 0.141                                     | 99.3                           | Do.                                  |                                                         |
| IV-A  | 0.025                     | C <sub>1</sub> /0.005 | 0                                 | 0.126                                     | 99.4                           | Do.                                  |                                                         |
| IV-A  | 0.050                     | C <sub>1</sub> /0.010 | 0                                 | 0.118                                     | 99.4                           | Do.                                  |                                                         |
|       |                           |                       | 0                                 | 0                                         | 20.936                         | 0                                    | Presents a dark brown color due to occurrence of smuts. |
| 25    |                           |                       |                                   |                                           |                                |                                      |                                                         |

TABLE 6.—CORROSION INHIBITING EFFECT  
[7% HCl, 70° C., 5 hr.]

| Type | Anticorrosive composition |                        | Corrosion rate, mg./cm. <sup>2</sup> /hr. | Inhibition efficiency, percent | Surface of processed steel coupon                       | Anticorrosive composition | Solubilizer/amount added, percent | Corrosion rate, mg./cm. <sup>2</sup> /hr. | Inhibition efficiency, percent | Surface of processed steel coupon |
|------|---------------------------|------------------------|-------------------------------------------|--------------------------------|---------------------------------------------------------|---------------------------|-----------------------------------|-------------------------------------------|--------------------------------|-----------------------------------|
|      | Amount added, percent     | Percent                |                                           |                                |                                                         |                           |                                   |                                           |                                |                                   |
| I    | 0.010                     | 0                      | 0.484                                     | 97.7                           | Maintains the original metal luster.                    | V                         | 0.010                             | 0                                         | 0.362                          | 98.3                              |
| I    | 0.025                     | 0                      | 0.209                                     | 99.0                           | Do.                                                     | V                         | 0.025                             | 0                                         | 0.277                          | 98.7                              |
| I    | 0.050                     | 0                      | 0.185                                     | 99.1                           | Do.                                                     | V                         | 0.050                             | 0                                         | 0.260                          | 98.8                              |
| I-A  | 0.010                     | A/0.002                | 0.277                                     | 98.7                           | Do.                                                     | V-A                       | 0.010                             | C <sub>1</sub> /0.002                     | 0.107                          | 99.5                              |
| I-A  | 0.025                     | A/0.005                | 0.213                                     | 99.0                           | Do.                                                     | V-A                       | 0.025                             | C <sub>1</sub> /0.005                     | 0.111                          | 99.5                              |
| I-A  | 0.050                     | A/0.010                | 0.170                                     | 99.2                           | Do.                                                     | V-A                       | 0.050                             | C <sub>1</sub> /0.010                     | 0.141                          | 99.3                              |
| I-B  | 0.010                     | B <sub>1</sub> /0.002  | 0.115                                     | 99.5                           | Do.                                                     | V-B                       | 0.010                             | C <sub>2</sub> /0.002                     | 0.196                          | 99.1                              |
| I-B  | 0.025                     | B <sub>1</sub> /0.005  | 0.111                                     | 99.5                           | Do.                                                     | V-B                       | 0.025                             | C <sub>2</sub> /0.025                     | 0.155                          | 99.3                              |
| I-B  | 0.050                     | B <sub>1</sub> /0.010  | 0.110                                     | 99.5                           | Do.                                                     | V-B                       | 0.050                             | C <sub>2</sub> /0.010                     | 0.136                          | 99.4                              |
| I-C  | 0.010                     | C <sub>1</sub> /0.002  | 0.111                                     | 99.5                           | Do.                                                     | VI                        | 0.010                             | 0                                         | 0.490                          | 97.7                              |
| I-C  | 0.025                     | C <sub>1</sub> /0.005  | 0.105                                     | 99.5                           | Do.                                                     | VI                        | 0.025                             | 0                                         | 0.405                          | 98.1                              |
| I-C  | 0.050                     | C <sub>1</sub> /0.010  | 0.084                                     | 99.6                           | Do.                                                     | VI                        | 0.050                             | 0                                         | 0.402                          | 98.1                              |
| I-D  | 0.010                     | B <sub>2</sub> /0.0030 | 0.113                                     | 99.5                           | Do.                                                     | VI-A                      | 0.010                             | C <sub>1</sub> /0.002                     | 0.284                          | 98.7                              |
| I-D  | 0.025                     | B <sub>2</sub> /0.0075 | 0.110                                     | 99.5                           | Do.                                                     | VI-A                      | 0.025                             | C <sub>1</sub> /0.005                     | 0.205                          | 99.5                              |
| I-D  | 0.050                     | B <sub>2</sub> /0.0150 | 0.097                                     | 99.5                           | Do.                                                     | VI-A                      | 0.050                             | C <sub>1</sub> /0.010                     | 0.103                          | 99.5                              |
| I-D  | 0.010                     | C <sub>2</sub> /0.002  | 0.133                                     | 99.3                           | Do.                                                     | VI-B                      | 0.010                             | C <sub>2</sub> /0.002                     | 0.306                          | 98.5                              |
| I-D  | 0.025                     | C <sub>2</sub> /0.002  | 0.109                                     | 99.5                           | Do.                                                     | VI-B                      | 0.025                             | C <sub>2</sub> /0.005                     | 0.237                          | 98.9                              |
| I-D  | 0.050                     | C <sub>2</sub> /0.010  | 0.095                                     | 99.5                           | Do.                                                     | VI-B                      | 0.050                             | C <sub>2</sub> /0.010                     | 0.167                          | 99.2                              |
|      | 0                         | 0                      | 20.936                                    | 0                              | Presents a dark brown color due to occurrence of smuts. |                           | 0                                 | 0                                         | 20.936                         | 0                                 |
| 55   |                           |                        |                                           |                                |                                                         |                           |                                   |                                           |                                |                                   |

## EXAMPLE 5

There were heated to 80° C. the 10% hydrochloric acid solutions to which there were added a prescribed amount

TABLE 9.—CORROSION INHIBITION EFFECT [10% HCl, 70° C., 5 hr.]

| Type                      | Number of days during which HCl remained mixed with anticorrosive compositions (80° C.) |                                   |                                           |                                |                                           |                                |                                           |                                |                                           |                                |
|---------------------------|-----------------------------------------------------------------------------------------|-----------------------------------|-------------------------------------------|--------------------------------|-------------------------------------------|--------------------------------|-------------------------------------------|--------------------------------|-------------------------------------------|--------------------------------|
|                           | 0 days                                                                                  |                                   | 5 days                                    |                                | 10 days                                   |                                | 30 days                                   |                                |                                           |                                |
| Anticorrosive composition | Amount added, percent                                                                   | Solubilizer/amount added, percent | Corrosion rate, mg./cm. <sup>2</sup> /hr. | Inhibition efficiency, percent | Corrosion rate, mg./cm. <sup>2</sup> /hr. | Inhibition efficiency, percent | Corrosion rate, mg./cm. <sup>2</sup> /hr. | Inhibition efficiency, percent | Corrosion rate, mg./cm. <sup>2</sup> /hr. | Inhibition efficiency, percent |
| I                         | 0.010                                                                                   | 0                                 | 0.690                                     | 97.3                           | 1.387                                     | 94.6                           | 2.020                                     | 92.2                           | -----                                     | -----                          |
| I                         | 0.025                                                                                   | 0                                 | 0.749                                     | 97.1                           | 1.189                                     | 95.3                           | 1.371                                     | 94.7                           | -----                                     | -----                          |
| I                         | 0.050                                                                                   | 0                                 | 0.752                                     | 97.1                           | 1.245                                     | 95.1                           | 1.438                                     | 94.4                           | -----                                     | -----                          |
| I-D                       | 0.010                                                                                   | C <sub>2</sub> /0.002             | 0.110                                     | 99.6                           | 0.120                                     | 99.5                           | 0.116                                     | 99.6                           | 0.403                                     | 98.5                           |
| I-D                       | 0.025                                                                                   | C <sub>2</sub> /0.005             | 0.105                                     | 99.6                           | 0.114                                     | 99.6                           | 0.131                                     | 99.5                           | 0.181                                     | 99.3                           |
| I-D                       | 0.050                                                                                   | C <sub>2</sub> /0.010             | 0.103                                     | 99.6                           | 0.115                                     | 99.6                           | 0.135                                     | 99.5                           | 0.136                                     | 99.5                           |
|                           | 0                                                                                       | 0                                 | 25.932                                    | 0                              | 25.514                                    | 0                              | 25.766                                    | 0                              | -----                                     | 0                              |

## 11

of the anticorrosive compositions of the Types I and I-D used in Example 1 as well as the solubilizer of the type C<sub>2</sub> used in Example 4. Said hydrochloric acid solutions were preserved at said temperature for 5, 10 and 30 days respectively. There were submerged, as in Example 1, a mild steel coupons for 5 hours in said solutions. There were made corrosion inhibition tests with said solutions maintained at 70° C. to determine the corrosion rate and inhibition efficiency and compare the high temperature stability of the respective anticorrosive compositions. The results are shown in the foregoing Table 9.

What we claim is:

1. A method of inhibiting the acid corrosion of metals which consists of inhibiting acid solutions from corroding metals by mixing with said acid solutions an anticorrosive composition prepared by the reaction of benzyl halides and materials mainly consisting of imidazoline derivatives having the following structural formula:



where:

R=group of alkyl, alkenyl or hydroxyalkenyl having 5 to 21 carbon atoms

m=0 or integer of 1 to 3

2. The method according to claim 1 wherein the benzyl halide is benzyl chloride.

3. The method according to claim 1 wherein the benzyl halide is benzyl iodide.

4. The method according to claim 2 wherein reaction of materials mainly consisting of imidazoline derivatives with the benzyl chloride is conducted at a temperature of 60 to 150° C.

5. A method of inhibiting the acid corrosion of metals which consists of inhibiting acid solutions from corroding metals by mixing with said acid solutions an anticorrosive composition prepared by the reaction of benzyl halides

5

10 where:

R=group of alkyl, alkenyl or hydroxyalkenyl having 5 to 21 carbon atoms

m=0 or integer of 1 to 3

and also mixing with said acid solution additives capable of rendering said anticorrosive composition soluble in said acid solutions.

15 6. The method according to claim 5 wherein the benzyl halide is benzyl chloride.

7. The method according to claim 5 wherein the benzyl halide is benzyl iodide.

8. The method according to claim 5 wherein the additives capable of rendering the anticorrosive composition soluble in acid solutions are selected from the group consisting of ethylene oxide addition products of higher alcohols, alkyl phenols and alkyl amines.

20 9. The method according to claim 5 wherein reaction of materials mainly consisting of imidazoline derivatives with the benzyl chloride is performed at a temperature of 60 to 150° C.

## References Cited

## UNITED STATES PATENTS

|           |        |                 |       |             |
|-----------|--------|-----------------|-------|-------------|
| 2,794,808 | 6/1957 | Albrecht et al. | ----- | 260—309.6   |
| 3,096,294 | 7/1963 | Hughes          | ----- | 260—309.6 X |
| 3,514,251 | 5/1970 | Annand et al.   | ----- | 21—2.7 R    |

30 35 MORRIS O. WOLK, Primary Examiner

T. HAGAN, Assistant Examiner

U.S. CL. X.R.

40 252—390; 260—309.6

## 12

and materials mainly consisting of imidazoline derivatives having the following structural formula:

